

## UNITED STATES PATENT OFFICE

2,146,630

## ALLOYS

John Johnson, Toronto, Ontario, Canada

No Drawing. Application June 6, 1938.  
Serial No. 212,135

## 4 Claims. (Cl. 75—155)

This invention relates to alloys such as described in my prior United States Patent No. 2,014,083 dated Sept. 10, 1935, and comprising silver, copper, cadmium and zinc substantially in the proportion of

|         | Per cent |
|---------|----------|
| Silver  | 33       |
| Copper  | 30       |
| Cadmium | 35       |
| Zinc    | 2        |

This alloy gives excellent results but the amount of silver employed makes the alloy rather expensive. Further, this alloy is not as successful as might be desired in brazing stainless steel to stainless steel or other metals.

My object therefore is to provide an alloy containing a smaller proportion of silver than heretofore used without materially affecting the desirable characteristics of the alloy and increasing its adaptability to the brazing of stainless steel.

I attain my object by decreasing the proportion of silver in the alloy and also the proportion of cadmium, at the same time increasing the proportion of copper and to a small extent the proportion of zinc.

In practice I have used silver, copper, cadmium and zinc within the following range of proportions:

|         | Per cent |
|---------|----------|
| Silver  | 7½ to 25 |
| Copper  | 62 to 40 |
| Cadmium | 19 to 31 |
| Zinc    | 9½ to 3  |

Specific examples of alloys according to my invention which I have tried are as follows:

| Example | Silver  | Copper  | Cadmium | Zinc    | Melting point |
|---------|---------|---------|---------|---------|---------------|
|         | Percent | Percent | Percent | Percent | ° F.          |
| No. 1   | 25      | 40      | 31      | 4       | 1076          |
| No. 2   | 18      | 48      | 31      | 3       | 1094          |
| No. 3   | 15½     | 48      | 31      | 5½      | 1076          |
| No. 4   | 12      | 58      | 21      | 9       | 1149          |
| No. 5   | 10½     | 57½     | 22      | 10      | 1124          |
| No. 6   | 9½      | 60      | 19      | 11½     | 1150          |
| No. 7   | 7½      | 62      | 21      | 9½      | 1150          |